

## UNITED STATES PATENT OFFICE

2,206,109

## COPPER-ZINC ALLOYS

Wolf Johannes Müller and Moritz Niessner,  
 Vienna, Germany, assignors to Oesterreichische  
 Dynamit Nobel Aktiengesellschaft, Vienna,  
 Germany, a firm of Germany

No Drawing. Original application June 25, 1938,  
 Serial No. 215,856. Divided and this applica-  
 tion July 1, 1939, Serial No. 282,522. In Austria  
 July 21, 1934

## 1 Claim. (CL. 75—155)

This invention is a division of our application  
 Ser. No. 215,856, filed June 25, 1938, for Copper-  
 zinc alloys.

It is known that gamma-brass, that is to say  
 copper-zinc alloys with a copper content of about  
 31-40%, i. e. alloys which are characterized by  
 a low copper content, are more resistant to cor-  
 rosion than the brass alloys of the alpha and  
 alpha and beta region with for instance 68-72  
 percent and more of copper, i. e., a higher cop-  
 per content. The technical employment of gam-  
 ma-alloys poor in copper is however impossible,  
 since these alloys are extremely hard and brittle  
 and are consequently not machinable.

From such alloys, as is described in our prior  
 Patents Nos. 2,006,598 and 2,006,599, it has been  
 disclosed that it is possible, by the addition of  
 a few percent of a metal soluble in gamma-brass  
 or alloyable therewith, such as nickel or, with  
 more advantage cobalt, preferably by a sim-  
 ultaneous addition of nickel and cobalt, to obtain  
 alloys, which possess the good resistance to cor-  
 rosion of gamma-alloys poor in copper, but are  
 also capable of being worked up, that is to say  
 can be treated with machine tools and can also  
 be rolled hot. Such alloys with an addition of  
 approximately 3-12% of cobalt, nickel or the  
 like individually or in mixture, that is to say for  
 instance pure copper-zinc alloys with a minimum  
 content of nickel of approximately 7-8% or of  
 cobalt of approximately 5-6% have extremely  
 good technical properties, and when cobalt and  
 nickel are used simultaneously it is possible with  
 30 a much smaller cobalt content to obtain the same  
 effects as with the use of cobalt alone. Conse-  
 quently alloys that are deficient in copper, even  
 those most deficient, can be made utilisable for  
 35 industrial purposes or as constructional material  
 for the production of articles, if the copper-zinc  
 alloys are alloyed with cobalt, nickel or the like  
 individually or in mixture.

The present invention is based on the ascer-  
 tained fact that such copper-zinc alloys, con-  
 40 taining between 30 and 45% of copper and be-  
 tween 3 and 12% of cobalt and/or nickel, can  
 have their properties substantially improved  
 when containing also between 4 and 15% of man-  
 gane 45 se and at least a small but effective amount  
 of one of the metals of the following group:

|           | Percent   |
|-----------|-----------|
| Iron      | Up to 1.8 |
| Aluminium | Up to 1.5 |
| Silver    | Up to 2.0 |
| Chromium  | Up to 3.0 |
| Tin       | Up to 2.0 |
| Lead      | Up to 0.3 |
| Selenium  | Up to 0.6 |
| Tellurium | Up to 0.6 |

10

but in no greater amounts than are soluble in  
 the solid solution and the zinc constituting sub-  
 stantially the remainder.

It has been ascertained that such alloys are  
 suitable for cold working, including cold rolling,  
 15 pressing and drawing and at the same time have  
 a high resistance to corrosion.

In carrying out the invention, the manganese  
 content should be smaller in the case of alloys  
 of higher copper content than in the case of alloys  
 of lower copper content. The higher the man-  
 gane 20 content the more suitable is the alloy for  
 cold working, a rising addition of manganese  
 up to about 10% leading to an approximately  
 proportional improvement in the cold working  
 25 properties.

By the addition of the metals of the group:  
 iron, aluminium, silver, chromium, tin, lead, se-  
 lenium and tellurium the workability in the cold,  
 the color and other properties of the alloys are  
 30 favourably influenced as compared with such al-  
 loys containing only copper, zinc, nickel and/or  
 cobalt and manganese as are subject of our co-  
 pending application Ser. No. 148,506, filed June  
 16, 1937.

Thus an enhanced workability in the cold can  
 be imparted to the alloys of the invention, by  
 the addition of suitable amounts of one or more  
 of the elements iron, lead, tin, selenium and  
 tellurium within the limits hereinbefore set forth  
 40 while their corrosion resistance can be enhanced  
 by the addition of one or more of the metals  
 aluminium, chromium and tin within the limits  
 hereinbefore set forth.

It is easy to ascertain empirically, the amount  
 45 of each element that will produce the most fa-  
 vorable effect.

A suitable alloy in accordance with the inven-  
 tion is one containing between 30 and 45% of  
 copper, between 3 and 12% of cobalt and/or  
 50

nickel, between 4 and 15% of manganese and between 0.5 and 1.5% of iron.

The addition of up to 0.3% of phosphorus to the herein-described alloys is advantageous since it very considerably improves the fineness of structure of the alloys.

By means of the additions according to the invention the range of the solid solution can also be increased, to some extent, beyond that

- 10. of the binary alloy, and alloys with a somewhat higher copper content which however must be substantially less than 45%, which come within the beta + gamma range in the binary alloy, can also be converted into a state corresponding to
- 15. gamma brass and rendered suitable for applications, such as cold rolling or drawing, from which they are otherwise excluded on account of their copper content.

The following is a typical example of an alloy according to the invention:

|           | Percent |
|-----------|---------|
| Cu.....   | 36      |
| Ni.....   | 6       |
| Co.....   | 2       |
| Mn.....   | 10      |
| Fe.....   | 1.2     |
| Zn.....   | 5       |
| Remainder |         |

What we claim is:

A corrosion-resistant copper-zinc alloy which is workable in the cold state, comprising copper 10 in the amount of 30 to 45%, at least one metal of the group cobalt and nickel in an amount of 3 to 12%, manganese in an amount of 4 to 15% and a small but effective amount of each of the following elements, iron up to 1.5% and silver 15 up to 2.0% to improve the fineness of grain of the alloy, the zinc constituting substantially all the remainder of the alloy.

WOLF JOHANNES MÜLLER.

MORITZ NIESSNER.

20